

## UNITED STATES PATENT OFFICE

LINN BRADLEY, OF MONTCLAIR, NEW JERSEY, AND EDWARD P. MCKEEFE, OF PLATTSBURG, NEW YORK, ASSIGNORS TO BRADLEY-MCKEEFE CORPORATION, OF NEW YORK, N. Y., A CORPORATION OF NEW YORK

## PROCESS OF PRODUCING PULP AND TREATMENT OF RESIDUAL LIQUORS

No Drawing.

Application filed May 9, 1928. Serial No. 276,501.

This invention relates to a process for producing pulp and treating residual liquor.

More particularly the invention relates to a process comprising digesting wood, etc., by means of a cooking liquor supplied with a sulfite of sodium, and digesting wood, etc., by means of cooking liquor supplied with sodium sulphide, some of the sodium content of residual liquor from one type of digesting treatment being utilized in cooking liquor of another type of digesting treatment.

According to one embodiment of the invention, we digest wood (for example, spruce or other coniferous or non-coniferous wood) by means of acid cooking liquor supplied with a sulfite of sodium, such digestion usually being carried out under conditions adapted to produce commercially bleachable chemical pulp; and we digest wood (for example, poplar, beech, birch, maple, pine or other wood) by means of alkaline cooking liquor supplied with sodium hydroxide and sodium sulfid (either with or without sodium sulfite being supplied thereto) usually conducting such digestion under conditions adapted to produce chemical pulp.

Residual liquor resulting from the acid digestion treatment is separated from the resulting fibrous material and is subsequently subjected to a concentrating treatment in any suitable manner, to remove water. The resulting residue is treated to decompose organic matter and to obtain some sodium sulfid including sulfur derived from a constituent of such residual liquor. Some of such sodium sulfid is subsequently employed in the alkaline cooking liquor referred to above.

Residual liquor resulting from the alkaline digesting treatment is separated from the resulting fibrous material and is subsequently subjected to a concentrating treatment in any suitable manner, to remove water, and the resulting residue is treated to decompose organic matter and to obtain some sodium carbonate including sodium derived from a constituent of such residual liquor. Some of such sodium carbonate is utilized in producing a sulfite of sodium and the latter is used in cooking liquor for the acid digestion treatment.

The following example will serve to illustrate how the invention may be carried out in practice, although the invention is not limited to such example, various modifications thereof being permissible without departing from the spirit and scope of the invention.

For the alkaline digesting treatment, around 10,000 pounds, bone-dry basis, of poplar or other suitable wood, etc., may be charged into a suitable digester and thereinto may be charged a suitable volume of aqueous cooking liquor containing around 1,700 pounds of sodium hydroxide (NaOH), more or less, and around 500 pounds of sodium sulfid (Na<sub>2</sub>S), more or less, and around 500 pounds of sodium sulfite (Na<sub>2</sub>SO<sub>3</sub>), more or less.

The cooking liquor may vary considerably in the amounts and proportions of such chemicals and the volume thereof may be anything suitable. The alkaline cooking liquor may be formed and the cooking operation may be carried out in any suitable manner, such for example as described in our U. S. Patent No. 1,651,665, dated December 6, 1927, or in one or more of our pending applications for Letters Patent, Serial Nos. 57,953 and 57,954, filed September 22, 1925, and Serial No. 120,514, filed July 3, 1926. Upon completion of the digesting operation, the resulting materials are discharged from the digester and the residual liquor is removed from the resulting fibrous material by any suitable means. It is advantageous to so conduct the digestion operation that the fibres of the resulting pulp are sufficiently strong, and yet readily bleachable, so that the bleached fibres may be supplied in relatively large amount in production of high quality book-papers.

The acid digesting treatment is carried out in a suitable digester, advantageously provided with a suitable acid-resistant lining. Around 10,000 pounds (bone-dry basis) of so-called hardwood (e. g. poplar, birch, maple, etc.) may be charged into such digester, and there may be also charged thereinto a suitable volume of aqueous cooking liquor supplied with around 2,000 pounds of so-

dium sulfite (calculated as  $\text{Na}_2\text{SO}_3$ ), more or less, and around 800 to 1,600 pounds excess  $\text{SO}_2$  (i. e. that over the amount calculated as present in  $\text{Na}_2\text{SO}_3$ ).

- 6 More or less than 2,000 pounds of sodium sulfite (as calculated above) may be supplied to such cooking liquor; and the ratio of free to combined  $\text{SO}_2$  may be suitably varied and regulated. When it is desired to obtain relatively strong chemical pulp which contains fibres that are readily bleachable to produce relatively strong high white fibres, such that they are suitable for being supplied in relatively large amount or proportion in producing high quality papers, in some cases it is advantageous to have the cooking liquor of such composition that it contains no excess  $\text{SO}_2$  beyond the sodium bisulfite ( $\text{NaHSO}_3$ ) stage, preferably having both 75
- 10  $\text{Na}_2\text{SO}_3$  and  $\text{NaHSO}_3$  in such cooking liquor in suitable amount and ratio. The cooking operation can be carried out as described in a co-pending application for U. S. Letters Patent, Serial No. 665,924, filed September 27, 1923, or any other suitable procedure may be adopted. The cooking liquor may be produced in any suitable manner, such for example as described in a companion or co-pending application, Serial No. 664,640, filed 80
- 15 September 24, 1923. Wood other than that specified, e. g. spruce, balsam, pine, etc., may be digested by means of such type of cooking liquor when a different fibrous material is desired.
- 20 35 Upon completion of the digesting operation, the resulting materials are discharged from the digester and the residual liquor is removed from the resulting fibrous material by any suitable means. It is advantageous to employ such a cooking liquor and to so conduct the digesting operation that the resulting pulp is largely made up of fibres which are relatively strong and yet readily bleachable, as indicated above, especially 85
- 25 40 when digesting so-called hardwood.
- 30 The residual liquors from the acid digesting treatment and the alkaline digesting treatment, respectively, may be treated separately, if desired, and the residual liquor 90
- 35 50 from the acid digesting treatment may or may not be neutralized or rendered alkaline to litmus prior to subjecting it to the concentrating treatment to remove water from it. It is advantageous, however, to treat the acid residual liquor so as to render it at least 95
- 40 55 neutral, and preferably alkaline to litmus, e. g. by treatment thereof with a reactive alkaline sodium compound or compounds. Such treatment of the acid residual liquor 100
- 45 60 may be used to regulate and control the proportion of sulfur present in sodium-bearing material resulting from decomposition of sodium-bearing organic matter by a furnacing treatment. For thus treating the acid 105
- 50 65 residual liquor, reactive sodium-bearing ma-

terial, such as that present in residual liquor from the alkaline digesting treatment or in soda recovered or derived from residual liquor, e. g. sodium carbonate or sodium sulfid or sodium hydroxide or mixtures of two or more of these compounds may be used in the required amount or amounts. Thus the acid residual liquor may be treated by slowly and gradually adding thereto, while the liquor is maintained hot (e. g. at or near the boiling point) and is being agitated to remove released gas, e. g.  $\text{CO}_2$ , the required amount of alkaline residual liquor to fix the free acid and provide a mixed liquor which has the desired degree of alkalinity (to litmus) such as to prevent its injuring iron parts of a multiple-effect evaporator at a point or points where the liquor comes in contact with it.

85 By proceeding in the manner outlined, some of the sodium carbonate of the alkaline residual liquor (which usually contains a small to moderate amount of sodium carbonate due to incomplete causticization when the alkaline cooking liquor was made) is utilized for reacting upon acid contained in the acid residual liquor. The resulting mixed liquor may contain some precipitated organic matter, resulting from decomposition of a sodium-organic compound of the alkaline residual liquor. Such precipitated matter may be removed from the liquor, in whole or in part, in any suitable manner, and such removed organic matter, etc., separately delivered into the furnace hereinafter referred to; or/and the mixed liquor may have added thereto a suitable sodium compound which is capable of redissolving the precipitated organic matter then present. Thus some causticized soda liquor may be added thereto in the required amount, or some sodium carbonate-sodium sulfid liquor may be thus used, or both causticized and uncausticized soda liquor may be thus employed so as to redissolve such precipitated organic matter as may then be present. In this manner the mixed liquor can be made ready and suitable for introduction into a multiple-effect evaporator, the precipitated organic matter having been removed in whole or in part and suitable alkali added to the liquor in such amount as will tend to minimize or prevent organic matter separating therefrom during treatment thereof in the evaporator, e. g. when such 110

90 100 evaporator contains iron tubes.

115 The mixed residual liquor, which may be prepared as above, is subjected to a concentrating treatment in a multiple-effect evaporator so as to obtain a concentrated mixed liquor, e. g. around 30 to 40° Baumé, more or less, and the concentrated mixed liquor is subjected to a further treatment to remove remaining water therefrom and the resulting dry residue is suitably furnace under reducing conditions so as to obtain a furnace prod-

uct which contains sodium carbonate and sodium sulfid. The ratio of these two compounds therein contained may vary somewhat depending upon the amounts and contents 5 of the residual liquors which have been mixed together and upon the amount of sulfur carried away by the furnace gases, etc. By using a much larger amount of soda in the alkaline residual liquor than that in the acid 10 residual liquor, i. e. the alkaline residual liquor added to the acid residual liquor containing a much larger amount of soda than that contained in the acid residual liquor, the furnace product derived therefrom usually 15 contains a larger amount of sodium carbonate than of sodium sulfid, and the furnace gases carry a substantial amount of sulfur-bearing material. When the amount of oxy-sulfur bearing material present in the mixed resid- 20 ual liquor is relatively high as compared to total soda, the chemically reduced furnace product derived therefrom usually contains a relatively large amount of sodium sulfid, although sodium carbonate may be present in 25 amount equal to or larger than that of the sodium sulfid. The reducing furnace used may be similar to those customarily employed in mills which operate the conventional so-called sulfate process, or rotary incinerators 30 of the soda process may be operated under reducing conditions.

The treatment of the concentrated liquor from the evaporator may be carried out in any suitable manner, employing any suitable 35 equipment; but we have found that such concentrated liquor may be sprayed or/and atomized into gases coming from the furnace, either directly from the furnace, or after passing auxiliary combustion chamber (if 40 any) operated in conjunction therewith, or after such gases have been passed through a steam boiler (following the combustion chamber) and used for generating steam and for effecting a partial cooling of the gases. 45 Such sprayed or/and atomized liquor undergoes an additional concentration as a result of such treatment. The mixed liquor, at suitable concentration, may be sprayed or/and atomized into the hot gases, as above 50 indicated, and thereby converted into a substantially dry finely divided material which includes a substantial amount of sodium organic matter, e. g. by atomizing highly concentrated residual liquor or mixed residual 55 liquor into such gases at around 200 to 400° F. (more or less). The resulting gases, including water vapor and suspended matter, may be passed into a high voltage electrical 60 precipitator so operated as to remove the substantially dry material from such gases, allowing the resulting gases and water vapor to pass onward as pointed out in a co-pending application, Serial No. 267,047, filed April 3rd, 1928. In this way a substantially dry 65 material is recovered from the gases.

Such dry material may thereafter be subjected to a reducing furnacing treatment, for example as disclosed in said co-pending application, thus producing a non-gaseous furnace product which includes sodium carbonate and sodium sulfid and also producing a gaseous product including sulfur-bearing material. By introducing a regulated amount of air into the auxiliary combustion chamber, the sulfur-bearing material of the gases is present mostly, if not all, in the form of oxy-sulfur material, e. g.  $\text{SO}_2$  or/and  $\text{SO}_3$  or a compound or compounds including such material or/and materials (e. g.  $\text{Na}_2\text{SO}_4$ ). When the resulting gases are treated as pointed out above, a large part of the oxy-sulfur bearing material (e. g.  $\text{Na}_2\text{SO}_4$ ) is removed from the gases along with the substantially dry finely divided material described above. By suitably regulating the amount of air supplied to the combustion chamber, the gases may carry a considerable amount of sulfur dioxide.

The gases which pass on from the spray chamber or chambers may contain sulfur dioxide which may be removed therefrom, e. g. by scrubbing such gases, at a point or points beyond the spray chamber or chambers and electrical precipitator (if any), referred to above, by means of suitable liquor, e. g. an aqueous solution comprising sodium carbonate or/and sodium sulfite, for instance soda liquor derived from the furnace product which has been treated to remove or eliminate sulfid-sulfur or to convert sodium sulfid thereof directly or indirectly into sodium sulfite. Thus a solution of the sodium compounds from the reducing furnacing operation may be treated to remove sulfid-sulfur therefrom, or/and to convert sodium sulfid directly or indirectly into sodium sulfite by a regulated oxidation treatment, such for example as described hereinafter or in co-pending applications for U. S. Letters Patent, Serial No. 686,137, filed January 14, 1924; Serial No. 248,960, filed January 23, 1928; Serial No. 266,863, filed April 2, 1928, and Serial No. 267,476, filed April 4th, 1928. Such a resulting solution may be used to scrub such gases to regain sulfur dioxide therefrom. The resulting solution, following the scrubbing operation, may be further sulfited, to such extent as needed or desired, and/or may be otherwise treated to prepare it for use in a digesting operation, e. g. one employing a sulfite of sodium type of cooking liquor.

We have found that the ratio of sodium sulfid to sodium carbonate in the reduced furnace product, referred to above, depends in part upon the ratio of sulfur to soda in the material which is charged into the reducing furnace and upon the amount of sulfur-bearing material removed by furnace gases; and, furthermore, upon the composition of the sul-

fur-bearing material in the material charged into the furnace. Thus, for a given ratio of sulfur to soda, in the charged material, it is desirable to have the included sulfur-bearing material contain a relatively large amount of an oxy-sulfur compound of sodium. Sodium sulfate appears to be more advantageous in the charge than sodium sulfite for the same total sulfur and soda contents in the charged material, as it seems to retain the sulfur with the soda more effectively, and thus provides a relatively higher sodium sulfid content in the reduced furnace product. Accordingly, by using an auxiliary combustion chamber into which a regulated amount of air is introduced, sulfur-bearing material in the gases may be converted, to a considerable extent, at least, into a sulfate condition, although by regulating the conditions, especially the air supply and the temperatures, the gases may also carry a considerable amount of  $\text{SO}_2$ .

After spraying concentrated residual liquor from a digesting operation into the gases, e. g. at a point or points beyond the steam boiler where the hot products of combustion have been used to produce steam, and after using an electrical precipitator to remove from warm gases resulting suspended solids in a relatively or substantially dry condition, the warm gases which pass beyond such precipitator may contain a sufficient amount of sulfur dioxide to justify scrubbing or otherwise treating them to regain sulfur dioxide. The amount of sulfur dioxide which may be present in such gases depends upon the conditions. For instance, if the material charged into the reducing furnace (e. g. a conventional smelting furnace) has a high content of sulfur as compared to soda, in a compound or compounds, such for instance as a sulfite of sodium or/and sulfo-organic matter, and also if the concentrated residual liquor, sprayed or/and atomized into the furnace gases at a point beyond the boiler, contains a relatively large amount of such sulfites, etc., such as residual liquor from the acid digesting operation described herein usually contains, the gases which are to be scrubbed may contain a very considerable amount of sulfur dioxide.

In operating a multiple-liquor mill according to the present process, it is advantageous to regulate the reducing furnacing treatment and the oxidizing treatment of the gases so that the gases beyond the combustion chamber contain considerable amounts of both sulfate and sulfite sulfur, and to remove from such gases substantially all of the sulfate sulfur, e. g. by spraying or/and atomizing residual liquor thereinto and removing a concentrated material, as pointed out above, and to leave in the gases a considerable amount of sulfur dioxide and to subsequently treat such gases to regain the sulfur dioxide and form a sulfite of sodium,

and to employ such sulfite of sodium in a cooking liquor of the sulfite of sodium type.

The furnace gases, after having passed through a suitable cooling means, for example, a steam boiler, may with advantage be passed through an electrical precipitator so operated as to remove from the gases the suspended solids such as sulfate of sodium, and to allow the  $\text{SO}_2$  to pass beyond. After the gases have been substantially freed from sodium sulfate and additional sulfate radical, if any, the residual sulfur dioxide-bearing gases are treated by means of sodium carbonate-sodium sulfite material, in solution, so as to regain such sulfur dioxide and to convert sodium carbonate into sodium sulfite. The latter sulfited soda-bearing material may be further adjusted or modified, as needed or desired, to prepare it for use in a cooking liquor of a sulfite of sodium type, etc.

The sulfate sulfur removed from such gases is later charged into the reducing furnace. In this method, the sulfate sulfur is utilized in an advantageous manner to provide a reduced furnace product of relatively high sodium sulfid content, which can, if desired, be advantageously employed in the alkaline cooking liquor of the process, and sulfite sulfur is regained from the gases and is employed, at least in part, in the sulfite of sodium type of cooking liquor. That is to say, we have found it desirable to conduct the recovery operations in such a manner as to provide a relatively high content of sodium sulfate in the material which is charged into the reducing furnace, some of such sulfate sulfur having been removed from gases derived from such furnace.

A sulfate of sodium, e. g. salt cake, can be added either to one or both of the types of residual liquors or to mixed residual liquor, or it can be added to the material which is to be charged into the reducing furnace, or it can be added to the material within such furnace. Thus sodium sulfate can be used to replace soda losses and also to supply some sulfur to the cycle, sodium sulfid being derived therefrom by a reducing treatment in the presence of incandescent carbon.

When the amount of residual liquor available from the alkaline type of digesting operation is sufficient, a portion of such residual liquor can be subjected to a suitable furnacing treatment (e. g. in a rotary incinerator) without having any other sulfur-bearing material added thereto. The furnace product which may be thus obtained, especially if the soda material has been given an oxidizing treatment, usually carries a relatively large amount of sodium carbonate as compared with sodium sulfid. When the amount of sodium sulfid in such furnace product is sufficiently low, an aqueous solution of the

soda thus recovered can be directly sulfited in any suitable manner to form cooking liquor for the sulfite of sodium type of digestion, i. e. an acid sulfite of sodium cooking liquor of the present process.

5 Such aqueous solution of the recovered soda may advantageously be used to regain sulfur dioxide from the furnace gases of either one or both of the above mentioned furnacing operations, such as by the method 10 pointed out above.

The portion of alkaline residual liquor which is to be subjected to such a separate furnacing treatment, if any, which may be 15 carried out in a conventional rotary incinerator, may be subjected to an evaporating treatment and may then be directly charged into a furnace of any suitable type, or it may be subjected to a spraying or/and an atomizing 20 treatment, in the manner pointed out, by means of gases which carry little or no sulfur-bearing material and the resulting concentrated material may be recovered and thereafter be charged into a suitable furnace 25 such as pointed out above or into any other suitable furnace. Such portion of the concentrated alkaline residual liquor may be treated in the manner and with the equipment used in the so-called Soda Process.

30 If desired, sodium carbonate can be added to the aqueous solution of the soda recovered in the furnace product which is to be sulfited, thereby replacing some of the soda losses; although when enough sulfate of sodium has 35 been added to the material which is to undergo the reducing furnace treatment, previously described, such addition of sodium carbonate can be dispensed with to advantage.

40 Owing to the fact that sulfate of sodium supplies sulfur as well as soda to the cycle a relatively small amount of additional sulfur is needed to replace losses thereof. This may be supplied in any suitable manner, 45 e. g. by burning sulfur in a sulfur-burner to provide  $\text{SO}_2$  and this may be used to form a sulfite of sodium or/and to increase the sulfite content of the solution which is to be utilized in preparation of the cooking liquor 50 of the acid type. By operating according to the methods outlined above, in which a large amount of sulfur is regained in useful condition, the amount of such newly supplied sulfur to be thus added is relatively small.

55 In case the aqueous solution which is to be sulfited to form a sulfite of sodium type of cooking liquor, e. g. the acid cooking liquor described above, contains such an amount of sodium sulfid as to render it objectionable or unsuitable for a direct sulfiting operation in which  $\text{SO}_2$  gas is introduced into a cold solution containing such an amount of sodium sulfid, the aqueous solution may be given a preliminary treatment prior to sulfiting it, e. g. by means of sulfur dioxide gas. In co-

pending applications we have described various methods of treating such an aqueous solution in order to obtain suitable sulfite of sodium cooking liquors, e. g. of the acid type. One or more of such methods, or any other 70 suitable method for treating such aqueous solutions to obtain suitable acid cooking liquor, may be employed, and the resulting cooking liquor used in a digesting operation.

75 Such a solution may be treated with an amount of zinc sulfite, or of zinc oxide, or advantageously of sodium zincate, such as will react with substantially all of the sodium sulfid to form insoluble zinc sulfid so as to remove substantially all sulfid-sulfur from 80 the solution. The treated solution is thereafter separated from the precipitate by any suitable means and the solution is thereafter subjected to such further sulfiting treatment 85 as desired or needed.

Alternately, sodium sulfid in such an aqueous solution may be treated with a suitable iron compound so as to remove the sulfid-sulfur in the form of precipitated iron sulfid, and the precipitated sulfid is thereafter removed from the solution by any suitable means. By mixing this precipitated and removed iron sulfid in proper amount with the soda bearing material which is to be charged into the reducing type of furnace, the resulting furnace product may be admixed with water and agitated and heated, if needed, and the resulting solution may be separated from the resulting iron sulfid by 90 any suitable means and in any suitable way.

95 A relatively insoluble alkaline-earth metal compound or compounds may be supplied to the mixture and it may be removed from the solution along with the iron sulfid so as to aid in separating a clear liquor. Thus basic magnesium carbonate in suitable amount may be so used, or other magnesium compounds may be used to clarify the liquor as described in our copending applications Serial Nos. 686,137 filed January 14, 1924, 704,176 filed April 4, 1924, and 713,257 filed May 14, 1924.

100 The solids removed from the liquor, e. g. a mixture of iron sulfid and the alkaline-earth metal compound or compounds, may be returned to the reducing furnace for treatment along with sodium-organic matter and sulfur-bearing material. The furnacing operation of the mixed charge should be so conducted and regulated that sulfur of the iron sulfid is driven out from its combination with the iron, e. g. into the furnace gases so as to provide oxy-sulfur-material in the gases beyond the combustion chamber. Such oxy-sulfur material can be regained from the furnace gases in a manner pointed out above. Instead of treating the iron sulfid precipitate, etc., along with another lot of sodium-organic matter, e. g. in the manner outlined above, such precipitate may be given a separate treatment in another furnace under condi- 110 115 120 125 130

tions adapted to form an iron compound (e. g. sodium ferrite) which is suitable for addition to the aqueous solution of the recovered sodium compounds and for reacting with 5 sodium sulfid thereof to form iron sulfid. In this way the sulfid-sulfur in the solution may be reduced to a suitable amount or it may be substantially eliminated therefrom.

- Sodium carbonate-sodium sulfid solution 10 may be treated with a suitable sulfate or sulfates so as to convert any desired portion or substantially all of the sodium content of the sodium sulfid and sodium carbonate into sodium sulfate and under conditions adapted 15 to remove sulfid-sulfur from the solution; then the sulfid-free (or substantially sulfid-free) solution may be thereafter treated in any suitable manner so as to convert sodium sulfate of the solution into a sulfite of sodium. 20 Thus the sodium carbonate-sodium sulfid liquor may be treated with ammonium sulfate or/and magnesium sulfate, or with calcium sulfate and magnesium sulfate or/and ammonium sulfate. Thus calcium sulfate 25 may be used to react upon a portion or all of the sodium carbonate and the other sulfate or sulfates may be used to react upon the sodium sulfid, and the solution may be heated (e. g. boiled) to remove therefrom substantially all liberated H<sub>2</sub>S. The latter may be 30 thereafter burned to form SO<sub>2</sub> which may be used to form a sulfite for use in a cooking liquor. The precipitated material, if any, may be removed from the solution before it 35 is treated with the sulfite radical. The sodium sulfate of the solution may be thereafter treated with calcium sulfite and excess SO<sub>2</sub> in amounts regulated so that calcium sulfate is formed as a precipitate, thus re- 40 moving from solution substantially all of the sulfate radical, and the sodium content of the sodium sulfate is converted into an acid sulfite of sodium in the solution. The acid solution is thereafter separated from the precipi- 45 tate and is then available as a cooking liquor or for preparation of cooking liquor.

All of the alkaline residual liquor, or any desired or necessary portion of it, may be admixed with the acid residual liquor and the 50 resulting mixed liquor treated as indicated above; or the two types of residual liquors may be treated separately so as to regain the soda in separate furnace products. The two types of residual liquors may thus be sepa- 55 rately treated by the spray evaporation treatment to form substantially dry materials.

These materials may be admixed in any desired ratio to form a mixture and the latter may be subjected to a furnacing treatment. 60 By regulating the amount of alkaline residual liquor admixed with acid residual liquor, and the ratio of soda to sulfur in the material charged into the reducing type of furnace, the ratio of sodium carbonate to sodium sulfid 65 can be regulated so as to give a regulated

range of composition of the solution of the recovered sodium compounds. In this way the causticized liquor for the alkaline cooking operation, obtained by treatment of the recovered soda solution with lime, can be varied in its ratio of sodium hydroxide to sodium sulfid. Some sodium sulfite may be added to or produced in such alkaline cooking liquor.

A regulated portion of the sodium carbonate-sodium sulfid solution may be treated with lime so as to provide the alkaline cooking liquor in desired amount, and another portion of it may be treated to remove sulfid-sulfur or/and to produce sodium sulfite including sodium content of such sodium sulfid. Such latter portion may be further treated so as to produce the acid cooking liquor for use in the process of the present invention.

A portion of the sodium carbonate-sodium sulfid solution, e. g. sufficient to provide the desired amount of sulfite of sodium which is to be employed in the acid cooking liquor, may be treated with sulfur dioxide bearing material while maintained at around the boiling point, in a suitable vessel such as a tank provided with an agitator as more fully described in our copending application Serial No. 267,476 filed April 4, 1928. Sulfur dioxide bearing gases, for example those obtained from the combustion chamber of a sulfur burner of the conventional type, may be gradually and slowly introduced into such solution at a point or points near the bottom of the tank in such manner and amount as to react with the sodium sulfid to drive out hydrogen sulfid from the solution and to convert most or substantially all of the sodium sulfid into either a carbonate of sodium or/and a sulfite of sodium without forming any large amount of sodium thiosulfate. The hydrogen sulfid removed from the solution can be delivered into a combustion chamber of a sulfur burner and therein burned to sulfur dioxide and the sulfite regained for reuse in cooking liquor; or such hydrogen sulfid can be delivered into a combustion chamber operated in conjunction with the reducing furnace into which sodium-organic material is charged, the hydrogen sulfid being thereby oxidized to an oxy-sulfur compound or compounds. Such oxy-sulfur material may be regained from resulting gases in the manner outlined above. In case sodium thiosulfate should be formed in objectionable amounts, the resulting material may be subjected to a regulated oxidizing as hereinafter described.

A simple and advantageous method for carrying the process of the present invention into practice comprises treating the acid residual liquor from the acid sulfite digesting treatment by means of sufficient reactive material (e. g. sodium carbonate-sodium sulfid liquor made by dissolving the recovered soda from the reduced furnace product) to render the

mixed liquor moderately alkaline to litmus, then mixing the resulting moderately alkaline residual liquor with the residual liquor from the alkaline digesting treatment, and charging this mixture of residual liquors into a multiple-effect evaporator to produce a concentrated mixed residual liquor.

The concentrated mixed residual liquor may then be treated to remove remaining water and the resulting residue may be furnace under reducing conditions in any suitable furnace to produce the furnace product which contains the sodium carbonate and the fairly large amount of sodium sulfid. The recovered soda may be dissolved in water to make a strong solution which contains sodium carbonate and sodium sulfid, and this latter solution may be divided into two or more parts. One of such parts can be causticized by means of lime to provide the alkaline cooking liquor (comprising sodium hydroxide and sodium sulfid, with or without sodium sulfite, etc.), and another of such parts may be directly sulfited at or around the boiling point, in a tank provided with an agitator, by means of available sulfur dioxide in amount sufficient to convert at least one-half and preferably more than one-half of the sodium sulfid directly into sodium sulfite. The hydrogen sulfid liberated and removed from the liquor may be delivered into a combustion chamber and therein burned to form sulfur dioxide or/and trioxide. Thus sulfur dioxide gas, which may be supplied in any suitable manner (for example as warm or hot sulfur-burner gases), may be introduced into the sodium carbonate-sodium sulfid liquor in amount sufficient and under conditions regulated so as to convert the desired amount of sodium sulfid into sodium sulfite and so as to avoid the formation of a commercially prohibitive amount of sodium thiosulfate in the liquor, as more fully described in our copending application for

45 U. S. Letters Patent, Serial No. 264,476 filed April 4, 1928.

The hydrogen sulfid liberated by such treatment is advantageously driven out from the solution substantially as fast as it is formed and such  $H_2S$  may with advantage be introduced into a combustion chamber operated in connection with the furnace in which the sodium organic compounds are decomposed to form the sodium carbonate and the sodium sulfid. In such combustion chamber the hydrogen sulfid is readily oxidized by oxygen of the gases and the resulting oxy-sulfur compound or compounds may with advantage be recovered from the resulting gases in a manner heretofore pointed out.

The sulfiting of the liquor may be terminated at any suitable time after the sodium sulfid has been decomposed and the hydrogen sulfid removed from the liquor with substantial completeness, or the sulfiting treatment

may be continued until the liquor contains a ratio of combined to uncombined  $SO_2$  rendering it suitable for the acid sulfite of sodium type of digesting treatment of the process.

By thus effecting the sulfiting of a portion of the sodium carbonate-sodium sulfid liquor at the boiling point of the liquor and while it is being vigorously agitated, the sulfite of sodium type of cooking liquor can be prepared in a simple and advantageous manner, thus permitting of a simple method of treating the residual liquors from both types of digesting operations, and the recovered soda can be divided into such portions as may be desirable in the process.

The strength of the sodium carbonate-sodium sulfid liquor may be anything suitable, but it is of advantage to have the solution of such strength that the respective cooking liquors can be produced without subjecting the liquor to an additional evaporating operation.

That portion of the sodium carbonate-sodium sulfid liquor which is to be sulfited, e. g. by free sulfur dioxide (and which may advantageously be supplied as

sulfur burner gases from a point beyond the combustion chamber so as to avoid the presence of elementary sulfur in the gases), is usually at a relatively high concentration so as to avoid having any very large amount of hydrogen sulfid present in the liquor at any time. Such solution may, for example, contain around 150 to 200 grams per litre, more or less, of sodium carbonate ( $Na_2CO_3$ ) and around 50 to 100 grams per litre, more or less,

of sodium sulfid ( $Na_2S$ ), and solutions which are almost saturated with such sodium compounds may be used, if desired, thereby reducing the amount of water present.

When hot sulfur burner gases of the type described are employed for the hot sulfiting treatment, some of the water of the solution may be evaporated thereby, thus producing a liquor of increased concentration or precipitating

out a compound of sodium, as the case may be. After completion of the sulfiting treatment, the liquor can be treated to prepare it for use in a digesting treatment. Some of the lime mud from the causticizing treatment

of a portion of the liquor may be used to clarify the liquor either before or after the sulfiting treatment, usually prior to the sulfiting treatment so as to avoid reacting upon uncombined  $SO_2$  by means of a reactive calcium compound.

When the sodium carbonate-sodium sulfid liquor is first treated with the available sulfur dioxide, e. g. by delivering  $SO_2$  gas into the liquor at a relatively slow rate and agitating the boiling liquor, little if any  $H_2S$  comes from the liquor. After a sufficient amount of  $SO_2$  has been absorbed, the  $H_2S$  is discharged from the liquor at an increasing rate until a maximum rate is reached. The  $H_2S$

continues to come from the liquor in copious

amounts until a large portion of the sodium sulfid has been reacted upon, after which the rate at which the  $H_2S$  comes from the liquor decreases and finally substantially ceases to 5 come from the liquor. At such time, the sulfur dioxide may be shut off from the tank and the tank may be continued under boiling conditions and the agitation continued to drive out some more  $H_2S$  which is then coming from the liquor at only a slow rate. After such continued treatment for a period of around a half-hour or so, the liquor may be given a further sulfiting, if desired, to 10 increase the amount of sulfite radicle therein 15 and so as to obtain any desired ratio of combined to uncombined  $SO_2$ . Such additional sulfiting, after removal of the hydrogen sulfid, may be effected in any suitable manner. For example, such resulting liquor (containing 20 sodium sulfite and usually containing some sodium carbonate) may be used to scrub gases from the furnacing operation to regain sulfur dioxide therefrom, when such gases contain sulfur dioxide in amount such as 25 to justify it; or the liquor may be sulfited in any other suitable manner and to any suitable degree.

The concentration of  $H_2S$  in the gases removed from the tank in which the sodium carbonate-sodium sulfid liquor is sulfited while boiling, will vary considerably depending upon conditions. When a rich  $SO_2$  gas (such for example as when  $SO_2$  from burner gases is absorbed in water or in a sodium sulfite solution and the free  $SO_2$  is later driven out therefrom) is used for the sulfiting of the sodium sulfid, the gases will usually be much richer in  $H_2S$  than when burner gases are directly used for the treatment of the sodium sulfid. The rich  $H_2S$  gases may be burned in a combustion chamber operated in connection with a sulfur burner, thus increasing the amount of  $SO_2$  in the gases. Diluted  $H_2S$  gases may be delivered into such a combustion chamber or they may be delivered into the combustion chamber of the furnace in which the sodium organic matter is decomposed.

Alternately the  $H_2S$  may be admixed with a suitable amount of air or/and  $SO_2$  and the mixed gases passed through a bed of suitably heated iron oxide or ferruginous bauxite under conditions regulated to selectively oxidize the hydrogen to form water vapor and 55 to leave the sulfur in the form of elementary sulfur. The latter may be recovered in molten condition in a manner well-known for the treatment of hydrogen sulfid.

In another method, the hydrogen sulfid, especially the dilute gases, may be scrubbed with a suitable solution of sodium carbonate to form a solution which contains both sodium acid carbonate and sodium acid sulfid ( $NaHCO_3$  and  $NaHS$ ) and the resulting solution may be subjected to a suitable aerat-

ing treatment to selectively oxidize the hydrogen to form water and to set free the elementary sulfur which can be removed from the resulting liquor in a manner understood. Such a method of treating dilute hydrogen sulfid gases has been described in connection with purification of illuminating and fuel gas. 70

When the hydrogen sulfid is delivered into a combustion chamber used in conjunction with a sulfur burner and when sulfur burner gases are used to treat the sodium sulfid in the liquor, the hydrogen sulfid may be delivered into a separate combustion chamber supplied with the portion of sulfur burner gases which is not used for treatment of the sodium sulfid, and another combustion chamber is used for producing the gases which are to be used for the treatment of the sodium sulfid. In this way building up of nitrogen, etc. to an objectionable point is largely obviated, although sulfur burner gases and combustion chambers are used. The sulfur dioxide-bearing gases are used in part for one treatment and in part may be used for further sulfiting of the partially sulfited liquor from the other treatment. 80

When a steam boiler is used in the manner indicated above to utilize heat from the furnace gases, the steam therefrom may be used in a multiple-effect evaporator to concentrate residual liquor, or/and in a digester in which wood is cooked by a cooking liquor of the present process. 95

In accordance with the present invention, a furnace product is obtained, e. g. by one of the methods heretofore outlined, which contains sodium carbonate and a relatively large amount of sodium sulfid. Such a furnace product may be obtained by mixing with the acid residual liquor just enough, or moderately more alkaline residual liquor than is required, to fix any free acid contained in the acid residual liquor, then subjecting the neutral or alkaline mixed liquor to a concentrating treatment including a spray evaporation treatment by means of furnace gases coming from a reducing furnace in which sodium-organic and sulfur-bearing materials are treated, such furnace gases preferably containing a considerable amount of sulfate sulfur, and recovering the resulting dried material by means of an electrical precipitator; then subjecting such dried material to a burning and reducing treatment in the furnace under conditions adapted to obtain the desired furnace product. Some of the sulfur content of the material charged into the furnace is usually eliminated into the furnace gases by such a furnacing treatment and the furnace product as obtained usually contains a considerable amount of sodium carbonate as well as sodium sulfid, the amount of sodium carbonate usually being larger than that of sodium sulfid. The furnace product is 100 105 110 115 120 125 130

treated with water to obtain a strong solution comprising sodium carbonate and sodium sulfid.

This solution may be cooled and thereafter directly sulfited by means of cool  $\text{SO}_2$  to form a relatively large amount of sodium thiosulfate therein, but leaving some of the sodium carbonate in such sulfited liquor. The sulfiting may thus be carried out under such conditions as to avoid driving out any considerable amount of sulfid-sulfur as hydrogen sulfid, it being preferable in this embodiment of the invention to retain all of the sulfur in the solution so as to obtain the maximum amount of thiosulfate. The sulfiting should usually be terminated when substantially all of the sulfid has been acted upon, although a small to moderate amount of sodium sulfite can be produced therein provided the required amount of sodium carbonate is left in the sulfited liquor.

The sulfiting of such a solution may be effected in any suitable manner. Thus such liquor (preferably rather cool) may be used to scrub cool furnace gases which carry sulfur dioxide, e. g. at a point beyond the electrical precipitator if any is used.

The resulting partially sulfited liquor, which contains a fairly large amount of sodium thiosulfate and still contains a considerable amount of sodium carbonate and may contain some sodium sulfite, is thereafter subjected to a regulated oxidizing treatment under conditions adapted to convert the sodium thiosulfate into sodium sulfite, some of the sulfur content of the thiosulfate being oxidized to sulfite and allowed to react with available soda to form sodium sulfite. Thus the sodium carbonate may be, at least in part, converted into sodium sulfite by means of the regulated oxidation of the thiosulfate, although the partially sulfited liquor may be given a regulated causticizing treatment, e. g. by means of lime, to convert a preponderating portion of the sodium carbonate into sodium hydroxide, prior to the regulated oxidation treatment to convert thiosulfate into sulfite. In case such a causticized liquor is thus used, the sodium hydroxide is, in part at least, converted into sodium sulfite due to oxidation of some of the sulfur content of the thiosulfate to sulfite.

Such regulated oxidation treatment of the partially sulfited liquor, referred to above, and either with or without previous treatment by means of lime (in the latter case the lime mud may be removed from the causticized liquor which contains the thiosulfate), may be effected in any suitable manner. For example, it may be treated to remove water therefrom to form a relatively dry finely divided soda-bearing material which includes thiosulfate and sodium carbonate or/and sodium hydroxide. Such material may have other suitable and finely divided solid mate-

rial, such as added sodium carbonate, sodium sulfite, carbon, calcium carbonate, etc. present therewith and quite uniformly distributed throughout it while it is being thus oxidized. Such finely divided material may be treated by means of air or other oxygen-bearing gases at a temperature ranging from around  $100^\circ \text{ C.}$ , up to around  $160^\circ \text{ C.}$ , more or less, usually around  $120^\circ$  to  $140^\circ \text{ C.}$ , so as to subject the finely divided material to suitable contact with a regulated and sufficient amount of oxygen to oxidize loosely combined sulfur of the thiosulfate to sulfite, and under conditions such that the formed sulfite radical may react with sodium carbonate or/and sodium hydroxide to form sodium sulfite.

The air or other oxygen-bearing gases for such treatment may be suitably heated to the desired point in any suitable manner and the oxygen-bearing gases may be caused to pass countercurrent to the soda-bearing material; or such gases and the soda-bearing material may be brought into intimate contact in any other suitable manner. Thus the material in suitably finely divided condition may be blown into, or the concentrated solution may be atomized into, the warm oxygen-bearing gases and allowed to react therewith to the desired extent and the treated solids may thereafter be removed from the residual gases by means of an electrical precipitator, for example. Or the suitably prepared soda-bearing material may be charged into a suitable furnace, such for example as a multiple-hearth furnace, and therein subjected to a progressive oxidation by means of such heated air brought into the lower part of such a furnace. Or the suitably prepared soda-bearing material may be spread out upon a traveling porous grate, such for example as a Dwight-Lloyd sintering machine, and suitably heated air may be caused to pass in a downward direction through the open and porous charge, thus subjecting the soda-bearing material to a regulated and progressive oxidation at suitable temperature as it travels from the charging end to the discharge end.

Upon completion of the oxidation of the thiosulfate to the desired degree, as indicated above, the resulting soda-bearing material may be dissolved in water in suitable amount and the resulting solution may be given such further sulfiting or other treatment as may be needed or desired to prepare the same for use in cooking liquor either for the acid type or for the alkaline type of digestion, or for both types. In the above embodiment of the invention, it is desirable to retain a relatively large amount of sulfur in the furnace product as sodium sulfide, and to use such material in forming a sulfite of sodium as pointed out.

The ratio of sodium hydroxide to sodium sulfid in the alkaline cooking liquor may be adjusted and controlled by mixing with liquor which is high in sodium sulfid a regulated

amount of liquor which is relatively high in sodium carbonate and low in sodium sulfid, such as may be obtained by a furnacing treatment of a regulated portion of the alkaline 5 residual liquor from the alkaline digesting operation, in a separate furnace, and without adding thereto any additional sulfur-bearing material. Thus in accordance with this embodiment of the invention, the sulfur content 10 of the sodium sulfid is used, at least to a considerable extent, in forming a sulfite of sodium and care is taken to avoid driving out sulfid-sulfur from the solution thereof as hydrogen sulfid.

15 In some cases, the treatment of sodium carbonate-sodium sulfid solution may be carried out with a combined sulfiting and oxidizing treatment. Thus the concentrated soda solution may be caused to pass countercurrent to 20 gases from a sulfur burner of such composition that they contain nitrogen, sulfur dioxide and a considerable amount of oxygen. Such gases may be cooled in any suitable manner, if needed, so that they are around 140 to 25 150° C., more or less, when they are brought into contact with a relatively dry and finely divided soda-bearing material. The oxygen of the gases serves to oxidize thiosulfate sulfur to sulfite sulfur, and the sulfur dioxide of 30 the gases serves to sulfite some of the sodium carbonate to form an oxy-sulfur compound of sodium. By regulating the composition, amount and temperature of such burner gases and regulating the composition and rate of 35 flow of the concentrated soda-bearing solution, and by adequate agitation and time for available sulfur to be oxidized to sulfite sulfur to the desired degree, the soda-bearing material removed from the discharge end of 40 the apparatus, in which the treatment is effected, may carry a relatively large amount of sodium sulfite and little if any thiosulfate. Such discharged material may be further sulfited or otherwise modified as needed or desired to prepare it for use in producing a type 45 of cooking liquor described above.

The following equations will serve to further illustrate various steps of treating 50 sodium sulfid to produce sodium sulfite by means of a regulated oxidation treatment at suitable temperatures as herein described.



60 The furnace product obtained as a result of the reducing furnace treatment, which contains sodium carbonate and sodium sulfid and usually with the former in preponderating amount, such for example as described above, 65 may be treated with a limited amount of

water so as to obtain a hot and highly concentrated solution of such sodium compounds. Such solution can be sprayed or atomized into a spray chamber and therein subjected to the evaporating action of hot gases which 70 contain a limited amount of oxygen, so as to obtain a relatively dry and finely divided soda-bearing material, and the resulting suspended matter can be removed from the moisture laden gases by passing the mixture 75 into a suitable electrical precipitator which is preferably operated at a temperature above the dewpoint of the moisture laden gases, the gases and contained moisture being allowed to pass beyond the precipitator. Such finely 80 divided and relatively dry or substantially dry soda-bearing material may thereafter be blown, for example, into a flue or chamber which is also supplied with heated air at a temperature ranging between 100° and 85 160° C., more or less, the usual temperature of such gases ranging advantageously between 120 and 140° C. The heated air may also have a small or moderate amount of steam therein to facilitate carrying out the 90 oxidation treatment. The finely divided material is thus brought into a highly disperse condition, in suspension in the gases, and excellent opportunity given for bringing the sodium sulfid and the oxygen into contact so 95 as to cause an oxidation of the sulfid-sulfur to form sulfite-sulfur, and the amount of oxygen allowed to react with sodium sulfid can be suitably regulated by controlling the amount of air and the amount of sodium 100 sulfid.

The oxidizing chamber is made of adequate size to permit the desired degree of oxidation being effected before the solids are removed from the gases. The treatment is 105 further improved by bringing the residual gases and suspended matter into an electrical precipitator and using a high voltage field between the electrodes to precipitate the solids from the gases. Care should be exercised to avoid heating the suspended matter and the air to a temperature so high that no moisture is present with the sodium sulfid and so high that most of the sodium sulfid is 110 oxidized to sodium sulfate, and the amount of air and its composition and its temperature should be suitably regulated so as to convert most of the sodium sulfid into sodium sulfate. Upon obtaining the desired conversion of sodium sulfid into sodium sulfite and to the desired degree, the oxidation is terminated so as to avoid producing an excessive amount of sodium sulfate such as might otherwise occur if the oxidation treatment 115 were continued for too long a time. By using an electrical precipitator after the oxidation chamber into which the sodium sulfid, etc., is introduced, the oxidized material can be promptly and effectively removed, thus 120 125 130

aiding in control of the regulated oxidation treatment.

By combining the evaporating and the oxidizing treatments, a further advantage is obtained. Thus the hot and concentrated sodium carbonate-sodium sulfid solution described above can be sprayed into hot oxygen-bearing gases under conditions to remove the desired portion of the moisture and a relatively dry material may thereby be oxidized to the desired degree. The oxidized material is then removed from the moisture laden gases in any suitable manner and by any suitable means, an advantageous means being, for example, an electrical precipitator.

By using a preponderating amount of sodium carbonate along with the sodium sulfid, the sodium sulfid is brought into a different condition for the oxidizing treatment thereof than when the sodium sulfid is in equal or preponderating amount as compared with sodium carbonate, etc., and the oxidation can be effected in an advantageous manner.

When the sodium carbonate-sodium sulfid material is to be directly subjected to a regulated oxidation treatment in a manner indicated above, there is the possibility that some of the sodium sulfid may be either underoxidized or overoxidized, e. g. into sodium sulfate, since it is usually preferable to overoxidize rather than to underoxidize and it is difficult in practice to control the oxidation so closely that only sodium sulfite is formed and yet oxidize all of the sodium sulfid.

We have found that the amount of sodium sulfate formed in such an oxidation treatment can be regulated to better advantage when the furnace product contains more sodium present as sodium carbonate than is present as sodium sulfid. Such a furnace product is readily obtained by treating the residual liquor in such manner that the excess sulfur is driven off in the furnace gases. The sodium carbonate and sodium sulfid are then to be subjected to a regulated oxidation treatment, in a manner pointed out above, and the resulting oxidized material containing sodium carbonate as well as sodium sulfite is employed to regain sulfur dioxide from the furnace gases, thus forming more sodium sulfite. By thus limiting and regulating the proportion of sodium sulfid in the furnace product and providing furnace gases which contain a relatively large amount of sulfur dioxide, the soda and the sulfur contents of the residual liquor can be, in rather large part, at least, regained in the form of sodium sulfite and without having formed too much sodium sulfate or/and sodium thiosulfate.

The residual liquor from the sulfite of sodium type of digestion, whether acid, neutral or alkaline (although any such acid residual liquor is customarily neutralized or/and

rendered alkaline to litmus, as stated above, prior to introducing it into the multiple-effect evaporator) is subjected to a regulated concentrating treatment in a multiple-effect evaporator, after which the concentrated liquor may be treated in the recovery apparatus of either the conventional soda process or the conventional sulfate process (so-called), under regulated reducing conditions, but with sufficient air being introduced into the furnace or furnaces so as to insure providing the kind of furnace gases described above (i. e. carrying such an amount of sulfur dioxide, etc.) and to provide a furnace product which carries more sodium present as sodium carbonate than as sodium sulfid, as pointed out. The melt from a sulfate process smelter, for example, may be treated with a small to moderate amount of water and the treatment continued under such conditions as will convert a preponderating amount of the sodium sulfid into sodium sulfite, usually oxidizing all or substantially all of the sodium sulfid either to sodium sulfite alone or in lesser part to sodium sulfate, and the resulting oxidized soda-bearing material may be used to regain sulfur dioxide from the furnace gases as described above.

If the recovery operation and equipment of the soda process are used, instead of those of the sulfate process, the furnacing is nevertheless carried out so as to obtain sodium sulfid and sodium carbonate, the sodium content of the later compound usually and advantageously being larger in amount than that of the former compound, and the furnace gases are provided with a relatively large amount of sulfur dioxide which may be regained therefrom by the soda-bearing material resulting from the regulated oxidation treatment of sodium sulfid referred to above. With the recovery operation of the soda process, as well as with that of the sulfate process, it is advantageous to remove and regain substantially all of the sulfate radical from the furnace gases prior to treating them with the oxidized soda-bearing material to regain sulfur dioxide therefrom.

The black ash formed when concentrated residual liquor, such as described above, is treated in the equipment of the soda process, e. g. under conditions to form a relatively large amount of sodium sulfid but with more sodium present in the black ash as sodium carbonate than is present therein as sodium sulfid, and to provide furnace gases with a relatively large amount of sulfur dioxide, may be treated with a small to moderate amount of steam so as to provide the sodium sulfid with a regulated amount of moisture, or the material may be otherwise treated with water for such purpose. For example, the black ash may be admixed with a small amount of water and agitated or ground

up in the presence of water to form a black ash slurry, and the slurry may be dried under conditions which leave the material finely divided. This finely divided material may then be thoroughly admixed with air of suitable temperature and in suitable amount to oxidize sodium sulfid thereof to sodium sulfite to the desired extent. Alternately, instead of treating the black ash in the foregoing manner, it may be finely ground in a relatively dry condition, either in the presence or absence of steam in regulated amount, and this finely ground relatively dry material may be subjected to the regulated oxidation treatment by means of the oxygen-bearing gases, such as air at suitable temperature, and which may also be supplied with a small to moderate amount of steam, either by drawing air through the mixture of carbon and the sodium compounds, or by agitating a mixture of air and such soda-bearing material, or by blowing such soda-bearing material into a chamber into which a suitable amount of air at suitable temperature is introduced, and the resulting oxidized material may be regained from residual gases in any suitable manner and by any suitable means. Such an intimate admixture of carbon and sodium compounds including sodium sulfid is advantageous, as it provides a relatively large surface to the air, etc., and facilitates oxidation thereof under suitably controlled and regulated conditions.

The process can also be used in pulp mills in which combinations of different liquors are used other than that described above, for example, mixed liquors containing sulfur compounds can be dried and furnaced as set forth herein, and the furnace product containing sodium carbonate and sodium sulfid treated with the sulfite radical to form a mixture of sodium carbonate and sodium thiosulfate. A portion of this liquor can be causticized and treated to form a cooking liquor containing sodium thiosulfate and caustic soda such as is described in our co-pending applications Serial No. 713,257, filed May 14, 1924, and Serial No. 705,711, filed April 10, 1924, and another portion subjected to a regulated oxidizing and treated to form a liquor containing a sulfite of sodium with or without some remaining thiosulfate. Liquors of these two types may be used in the cooking of wood and the resulting residual liquors mixed and regenerated according to the present invention. In some cases it may be found desirable to causticize sodium carbonate remaining in the thiosulfate containing liquor. A portion of this causticized liquor may be used directly to form a cooking liquor and another portion then subjected to a regulated oxidizing to form a cooking liquor containing a sulfite of sodium or sodium sulfite and caustic soda as set forth in co-pending applications referred to above.

The present application is a continuation in part of our co-pending applications Serial Nos. 133,289; 133,291, and 133,292 filed September 2, 1926, Serial No. 248,960 filed January 23, 1928, as well as the applications referred to in the foregoing specification. <sup>70</sup>

We claim:—

1. The cyclic process of producing pulp from wood, etc., which comprises digesting one lot of such fibrous material in a liquor containing a sulfite of sodium, digesting another lot of fibrous material in a liquor containing sodium hydroxide, separating a residual liquor from resulting fibrous material from each of such digesting treatments, removing water from such residual liquors, decomposing sodium organic compounds of both residual liquors furnacing them together, thereby producing a furnace product comprising sodium carbonate and sodium sulfid, causticizing a portion of the sodium carbonate thus recovered to form a cooking liquor comprising sodium hydroxide, introducing available sulfur dioxide into a hot solution that contains a substantial portion of the sodium carbonate and a substantial portion of the sodium sulfid, thus recovered, thereby removing hydrogen sulfid from the solution and converting some of the sodium content of the sodium sulfid and of the sodium carbonate into a sulfite of sodium and forming a cooking liquor comprising such sulfite of sodium, digesting fibrous material with each of such cooking liquors, and repeating the process. <sup>75</sup>

2. The cyclic process of producing pulp from raw cellulosic fibrous material, which comprises digesting one lot of such fibrous material in a liquor containing a sulfite of sodium, digesting another lot of such fibrous material in a liquor containing sodium sulfid, separating a residual liquor from resulting fibrous material from each of such digesting treatments, removing water from such residual liquors, decomposing sodium organic compounds of both residual liquors together by means of the same furnacing treatment, thereby producing a furnace product comprising sodium carbonate and sodium sulfid, forming a cooking liquor comprising a portion of the recovered sodium sulfid, treating another portion of the recovered sodium carbonate and sodium sulfid to form a sulfite of sodium and forming a cooking liquor comprising such sulfite of sodium, digesting fibrous material with each of such cooking liquors, and repeating the process. <sup>100</sup>

3. The cyclic process of producing pulp from raw cellulosic fibrous material, which comprises digesting one lot of such fibrous material in a liquor which is acid to litmus and contains the sulfite radicle, digesting another lot of such fibrous material in a liquor containing a reactive compound of sodium sulfite, and repeating the process. <sup>105</sup>

um alkaline to litmus, separating a residual liquor from resulting fibrous material from each of such digesting treatments, treating the residual liquor from the first-mentioned 5 digesting treatment by means of an alkaline sodium compound derived from the second-mentioned digesting treatment, removing water from the treated residual liquor, decomposing organic matter thereof under 10 conditions adapted to produce a furnace product comprising sodium carbonate and sodium sulfid, introducing available sulfur dioxide into a hot solution that contains a portion of such recovered sulfid to form and 15 remove hydrogen sulfid and to form a sulfite of sodium, forming a cooking liquor comprising such formed sulfite, digesting fibrous material with such cooking liquor, and employing the resulting residual liquor in re- 20 peating the process.

4. The cyclic process of producing pulp from raw cellulosic fibrous material, which comprises digesting one lot of such fibrous material in a liquor which is acid to litmus 25 and contains a sulfite of sodium, digesting another lot of cellulosic fibrous material in a liquor containing sodium hydroxide and sodium sulfid, separating an acid residual liquor from resulting fibrous material of the 30 first-mentioned digesting treatment, separating an alkaline residual liquor from resulting fibrous material of the second-mentioned digesting treatment, treating the acid residual liquor with an alkaline sodium compound de- 35 rived from the alkaline liquor, removing water from the resulting liquor, decomposing sodium organic matter thereof under conditions adapted to form a furnace product comprising sodium carbonate and sodium sulfid, adding lime to a liquor that contains some 40 of such recovered sodium carbonate and sodium sulfid and causticizing a portion of the sodium carbonate thus recovered to form a cooking liquor comprising sodium hydroxide and sodium sulfid, introducing available sulfur dioxide into hot liquor that contains a portion of the recovered sodium carbonate and sodium sulfid and thereby sulfiting a portion of the recovered sodium carbonate 45 and sodium sulfid under conditions adapted to produce a cooking liquor which contains a sulfite of sodium derived in part from the sodium carbonate and in part from the sodium sulfid, digesting such fibrous material 50 by means of each of such cooking liquors, and repeating the process.

5. The process according to the preceding claim, wherein acid residual liquor is rendered non-acid to litmus by adding thereto a 55 regulated amount of sodium carbonate and sodium sulfid derived from the furnacing step of the process.

6. The process according to claim 4, wherein a portion of the sodium carbonate and sodium sulfid of the furnace product is treated

in aqueous solution with available sulfur dioxide while the liquor is maintained at around the boiling point, thereby forming hydrogen sulfid and removing it from the solution and producing a sulfite of sodium that includes 70 sodium derived from the sodium sulfid.

7. The process according to claim 4, wherein a portion of the sodium carbonate and sodium sulfid of the furnace product in aqueous solution is treated while boiling, with 75 sulfur dioxide gas, thereby forming hydrogen sulfid and removing it from the solution and producing a sulfite of sodium that includes sodium derived from the sodium sulfid.

8. The process according to claim 4, wherein a portion of the sodium carbonate and sodium sulfid of the furnace product in aqueous solution is treated while boiling with sulfur dioxide gas supplied as sulfur-burner gases substantially free from elementary sulfur, 80 thereby forming hydrogen sulfid and removing it from the solution and producing a sulfite of sodium that includes sodium derived from the sodium sulfid.

9. The process according to claim 4, wherein in the sodium organic compounds from both types of residual liquors are furnaced together to produce a furnace product comprising sodium carbonate and sodium sulfid.

10. The method of producing pulp from fibrous material which comprises digesting cellulosic fibrous material in a liquor containing most of its sodium content in the form of a sulfite of sodium, treating cellulosic fibrous material in a liquor that contains most of its sodium content as alkaline sulfur-free compounds comprising sodium hydroxide, separating a residual liquor resulting from each of such treatments, mixing such residual liquors in suitable proportions, subjecting the mixture to a treatment adapted to recover sodium compounds thereof as sodium carbonate and sodium sulfid, such treatment including a reducing furnacing treatment, causticizing a portion of the recovered soda product and forming therefrom a liquor that contains most of its sodium content as alkaline sulfur-free compounds comprising sodium hydroxide, introducing 95 sulfur dioxide into a solution that contains a portion of the recovered sodium carbonate and sodium sulfid thereby sulfiting a portion of the recovered soda to form a product containing a tri-oxy-sulfur compound of sodium 100 and forming a cooking liquor therefrom suitable for use in the first named cooking treatment.

11. The method according to claim 10, in which a portion of the recovered soda product is treated with the sulfite radical until substantially all of the sodium sulfid in such portion is converted into tri-oxy-sulfur compound of sodium and the resulting product is subjected to a regulated oxidizing treat- 105 110 115 120

125 130

ment adapted to oxidize sodium thiosulfate to a sulfite of sodium.

12. The method according to claim 10, wherein the product containing sodium thiosulfate is subjected to a regulated oxidizing treatment whereby substantially all of the thiosulfate is converted into a sulfite of sodium.

13. The method of producing pulp from fibrous material which comprises digesting cellulosic fibrous material in an acid liquor containing sulfite of sodium, treating cellulosic fibrous material in a liquor that contains most of its sodium content in the form of alkaline sodium compounds comprising sodium sulfid, separating a residual liquor resulting from each of such digesting treatments, mixing such residual liquors in suitable proportions and subjecting the mixture to a treatment adapted to recover sodium compounds thereof as sodium carbonate and sodium sulfid, such treatment including a reducing furnacing treatment, causticizing a portion of the recovered soda product and forming thereof a cooking liquor for use in the alkaline cooking treatment, sulfiting a portion of the recovered soda product to convert substantially all of the sodium sulfid into tri-oxy-sulfur compounds of sodium containing at least some thiosulfate, subjecting the resulting product to a regulated oxidizing treatment until substantially all of the sodium thiosulfate has been converted into a sulfite of sodium and treating the resulting product to form a cooking liquor adapted for use in the acid cooking treatment.

14. The process according to claim 13, in which gases from the reducing furnace are oxidized to convert sulfur containing material therein into sulfur dioxide and sulfur trioxide, separating sulfur trioxide containing material from the gases and returning it to the reducing furnace and utilizing the sulfur dioxide for treating sodium compounds recovered from the reducing furnace in the preparation of the acid cooking liquor, and digesting cellulosic fiber-bearing material with the cooking liquor thus produced.

15. The cyclic method of treating cellulosic fiber-bearing material including lignous matter, which comprises digesting such material with cooking liquor that contains most of its sodium content in the form of oxy-sulfur compounds comprising a sulfite of sodium and a thiosulfate, treating cellulosic fiber-bearing material by means of an alkaline liquor that contains sulfur-free alkaline compounds of sodium and also contains sodium sulfid, separating a residual liquor that includes organic matter from fibrous material resulting from each of said treatments, removing water from such residual liquors, subjecting together sodium compounds derived from both of such residual liquors to a furnacing treatment under re-

ducing conditions thereby forming furnace gases that carry sulfur oxides and also forming another furnace product that contains most of its sodium compounds as sodium carbonate and sodium sulfid, dissolving such recovered sodium compounds in water, separating such alkaline solution into portions, introducing into one of such portions a sufficient amount of available sulfur dioxide to convert substantially all of the sodium content of the sodium carbonate and the sodium sulfid thereof into a sulfite of sodium and a thiosulfate of sodium, digesting cellulosic fiber-bearing material including ligneous matter by means of cooking liquor containing the sulfite of sodium and the thiosulfate of sodium thus produced, and treating cellulosic fiber-bearing material with an alkaline liquor that includes sodium sulfid contained in another of said portions and also includes an alkaline sulfur-free sodium compound, and repeating the process.

16. The further improvement in the method of claim 15, in which the first-mentioned cooking liquor is non-acid to litmus and the amount of sodium sulfite is larger than the amount of sodium thiosulfate therein.

17. The further improvement in the method of claim 15, in which one of the said portions of the alkaline solution is treated with lime to convert sodium carbonate into sodium hydroxide, and the resulting solution that contains sodium hydroxide and sodium sulfid is used to treat cellulosic fiber-bearing material, thereby forming an alkaline residual liquor that contains organic matter derived from the fiber-bearing material.

18. The further improvement in the method of claim 15, in which residual liquor from the first-mentioned digesting treatment is sprayed into hot gases formed during the furnacing treatment, thereby producing a substantially dry product that contains sodium-organic compounds, removing such dried material from the gases, and subjecting such dried material to a burning and reducing treatment in the furnace in which the said hot gases are formed.

19. The further improvement in the method of claim 1 in which the hydrogen sulfid removed from the solution is introduced into a combustion chamber operated in connection with the furnace in which the sodium organic compounds are decomposed and the sodium carbonate and sodium sulfid are produced.

In testimony whereof we affix our signatures.

LINN BRADLEY.

EDWARD P. MCKEEFE.

125

130